

# UNITED STATES PATENT OFFICE.

RUSSELL S. PENNIMAN AND JOHN C. SCHRADER, OF DOVER, NEW JERSEY,  
ASSIGNORS TO THE ATLANTIC DYNAMITE COMPANY, THE REPANNO  
CHEMICAL COMPANY, AND THE HERCULES POWDER COMPANY.

## DYNAMITE.

SPECIFICATION forming part of Letters Patent No. 333,149, dated December 29, 1885.

Application filed January 22, 1885. Serial No. 153,600. (No specimens.)

To all whom it may concern:

Be it known that we, RUSSELL S. PENNIMAN and JOHN C. SCHRADER, both of Dover, in the county of Morris and State of New Jersey, have invented certain new and useful Improvements in Explosive Compounds; and we do hereby declare that the following specification is a clear, true, and complete description of our invention.

10 The object of our present improvement is to lessen the cost and increase the specific gravity of nitro-glycerine compounds known as "ordinary dynamites," and containing finely-communited solid matters, by which the 15 nitro-glycerine is controlled, the whole being a practically adhesive or plastic mass. It is well known that in all compounds of this class the nitro-glycerine is the most expensive element, and it is equally well known that much 20 attention has heretofore been given to the production of more or less serviceable compounds containing said liquid explosive in such reduced proportions as would indicate apparent economy in their use.

25 In accordance with our invention, we can employ any one of these prior compounds containing solid combustible matter, or mixtures of any two or more of them, or we can employ the well-known mixtures of nitro-glycerine and infusorial earth, in which the earth is relied upon merely as a vehicle for properly controlling the liquid explosive or holding it in suspension; and for the purpose of illustrating the general value of our improvement we will first describe it in connection 30 with said earthy compounds, although for obtaining the best results the solid matter should be composed of combustible materials. Of a seventy-five per cent. compound of nitro-glycerine and earthy matter, we take, say, forty parts, and mix these with sixty parts of protected nitrate of ammonia, and produce a compound of greater specific gravity and of much greater effective force than said seventy-five 40 per cent. earth compound and at about twelve and one-half per cent. less cost. We do not, however, deem it desirable to employ non-combustible solid matter, because the best results involve the use of such well-known com-

bustible matters as have been heretofore employed in the manufacture of "dope" used in nitro-glycerine compounds—as, for instance, coal of various kinds, niter, nitrate of soda, and sulphur, whether such materials have been ground together and then mixed in mass with the nitro-glycerine, or first formed into small or fine composite grains, and then mixed with the liquid explosive, it being understood that our present invention contemplates the use of any of the ordinary types of dynamite, which in mass are clingy, pasty, or plastic, because of the presence of such a proportion of the liquid explosive as to coat or cover the particles or grains of solid matter with said explosive.

50 Among the great variety of what may be termed "ordinary dynamites," we will mention the plastic or adhesive mixtures of powdered charcoal, wood fiber, nitrate of soda, and sulphur, charged with from fifteen to seventy-five or eighty per cent. of the liquid explosive.

55 In producing our compounds we vary the proportion of such dynamites to the protected nitrate of ammonia according to the character of the service intended to be performed, it being understood that in all cases there must be sufficient nitro-glycerine to insure detonation throughout the mass, and for accomplishing this end our compounds should seldom, if ever, contain less than eighteen or twenty per cent. of the liquid explosive—as, for instance, in using a twenty-five per cent. dynamite containing either or all of the solid combustible matter enumerated, we add to seventy parts of such dynamite thirty parts of the protected nitrate of ammonia for producing a desirable compound of comparatively low grade, but superior in effective force to any ordinary dynamite containing as much as forty per cent. of the liquid explosive. This compound will be found to have a much greater specific gravity than any forty per cent. dynamite, and it can be produced at about eight-tenths of the cost thereof.

60 For producing a highly effective and economical compound, we combine with fifty parts of seventy-five per cent. dynamite fifty parts

65

70

75

80

85

90

95

of the protected nitrate. This compound will possess greater effective force than the seventy-five per cent. dynamite, and will have greater specific gravity, and it can be produced at about one-seventh less cost. The nitrate of ammonia must be thoroughly dehydrated in granular form, and each grain jacketed with an envelope or coating of soft or viscous carbonaceous matter for which nitro-glycerine has no affinity, and we prefer to use what we will term "Penniman's Protected Nitrate of Ammonia," which for the purposes of this specification may be described as grains of said nitrate coated with petroleum or its soft educts or products, preferably cosmoline. If said particular protected nitrate be not readily available, it can be prepared in its best form by thoroughly mixing with a given quantity of carefully-dehydrated granulated nitrate of ammonia from eight to twelve per cent. of cosmoline.

We are aware that it has been heretofore proposed to employ nitrate of ammonia in nitro-glycerine compounds—as, for instance, as set forth in the English Letters Patent of Nobel, No. 1,570 of A. D. 1873, wherein it is also suggested that by grinding paraffine with the nitrate of ammonia and charcoal the nitrate will be protected from deliquescence, and it is to be distinctly understood that any compounds in which such solid protecting agents are employed as require to be ground with the nitrate of ammonia are wholly outside of our present invention.

We are also aware that the English provisional specification No. 2,420 of 1876, suggests in a general way the use of nitrate of ammonia in explosive compounds, and the protection of the nitrate by the use of melted paraf-

fine or stearine or other similar solid bodies, all of which we wholly disclaim, because we are well aware that unless the grains of nitrate of ammonia have a soft or viscous coating its use in any explosive compound cannot be relied upon for producing practically desirable results.

It is to be understood that our present application does not relate to nitro-glycerine compounds embodying solid matters which are in the form of absorbent composite combustible grains, and which may be termed "grained dynamites," as distinguished from the "ordinary dynamites," which are wet and plastic because of the finely-communited condition of the solid matter by which the flowing propensities of the nitro-glycerine are controlled. It is also to be understood that our present application does not relate to compounds of gelatinized nitro-glycerine and nitrate of ammonia, in which the latter is not specially protected, as described in the English Letters Patent of Nobel, No. 4,179 of 1875.

Having thus described our invention, we claim as new and desire to secure by Letters Patent—

An explosive compound, substantially as hereinbefore described, containing finely-communited solid matter charged with nitro-glycerine and grains of nitrate of ammonia, which are inclosed within a soft or viscous envelope or coating for which nitro-glycerine has no affinity, as set forth.

RUSSELL S. PENNIMAN.  
JOHN C. SCHRADER.

Witnesses:

WM. S. WHITE,  
JAS. H. NEIGHBOUR.